



## EXAMPLE 4

 $\beta$ -Cyanovinyl-N-benzyl-N-methyldithiocarbamate

By following the procedure of Example 3 except for the substitution of an equimolar quantity of sodium N-benzyl-N-methyldithiocarbamate for the dithiocarbamate used therein, the product  $\beta$ -cyanovinyl-N-benzyl-N-methyldithiocarbamate can be obtained.

## EXAMPLE 5

## Flotation of a copper ore

In order to show the utility of the dithiocarbamates of the present invention as flotation promoters, the compounds of Examples 1, 2 and 3 were employed in the recovery of copper from an ore from the western United States, using the following procedure. The ore sample was ground for 5 minutes at 60% solids with 0.03 lb./ton of promoter (pH 7.8). It was then conditioned for one minute with 0.09 lb./ton of cresylic acid and 0.025 lb./ton of fuel oil. The pulp was floated for 8 minutes and the tailing analyzed for residual copper, with the following results.

TABLE I

| No.    | Compound       | Percent Cu in tailing |
|--------|----------------|-----------------------|
| 1..... | Example 1..... | 0.19                  |
| 2..... | Example 2..... | 0.34                  |
| 3..... | Example 3..... | 0.19                  |

I claim:

1. The process of beneficiating sulfide ores having copper values, which comprises subjecting the ore to froth-

flotation in the presence of a flotation promoter of the general formula:



wherein R and R' are individually selected from the group consisting of alkyl of up to eighteen carbons, containing up to about three substituents selected from the group consisting of chloro, bromo, fluoro, nitro, cyano, lower alkoxy and amino; phenyl, naphthyl and diphenyl having up to about five substituents selected from the group consisting of chloro, bromo, fluoro, lower alkyl, cyano, amino, nitro and lower alkoxy; and benzyl and naphthylmethyl having up to about three substituents selected from the group consisting of chloro, fluoro, bromo, lower alkyl, cyano, lower alkoxy, amino and nitro.

10 2. The process of claim 1 wherein the flotation promoter is  $\beta$ -cyanovinyl diethyldithiocarbamate.

15 3. The process of claim 1 wherein the flotation promoter is  $\beta$ -cyanovinyl di-n-butylthiocarbamate.

## References Cited by the Examiner

| 25 | UNITED STATES PATENTS |         |                             |
|----|-----------------------|---------|-----------------------------|
|    | 2,854,467             | 9/1958  | Harman et al. ----- 260—455 |
|    | 2,901,498             | 8/1959  | Tilles et al. ----- 260—455 |
| 30 | 2,914,457             | 11/1959 | Gaertner ----- 260—455 X    |

HARRY B. THORNTON, Primary Examiner.

R. HALPER, Assistant Examiner.